

## UNITED STATES PATENT OFFICE

2,030,739

## PROCESS OF PRODUCING SILICON-RAYON

Rudolph S. Bley, Elizabethton, Tenn., assignor to  
 North American Rayon Corporation, New York,  
 N. Y., a corporation of Delaware

No Drawing. Application October 22, 1934,  
 Serial No. 749,488

## 8 Claims. (Cl. 106—40)

The present invention relates to a process of preparing cellulosic spinning solutions from which soft-lustre products, such as filaments, yarns, ribbons, films, etc., may be produced.

5 The primary object of my invention has to do with the incorporation of aliphatic silicon compounds into cellulosic spinning solutions, such as viscose and cuprammonium cellulose, which will yield upon extrusion or molding soft-lustre products of pleasing hand.

10 Another object of my invention relates to the admixture of silicon compounds, having the structure  $R.SiH_3$  in which R represents an alkyl radical, with viscose and cuprammonium cellulose.

15 A third object of my invention has to do with the incorporation of silicon compounds into viscose and cuprammonium cellulose solutions, said compounds having the structure  $R.SiH_3.OH$  in which R represents an alkyl radical.

20 A fourth object of my invention has to do with the dispersion of silicon compounds in the aforementioned cellulosic solutions, these compounds having the structure  $R.SiH(OH)_3$  in which R represents an alkyl radical.

25 A fifth object of this invention relates to the formation of novel, soft-lustre products per se containing aliphatic silicon compounds.

30 Other objects of my invention will become apparent to those skilled in the art after a study of the following specification.

In the early days of rayon manufacture, the demand was entirely for yarns having the highest possible degree of lustre. Later, when it was found that highly lustrous rayon too clearly indicated its origin—an artificial fibre—a demand arose for artificial silk which more closely approximated to natural silk. The earliest attempt to meet the demand of dull-lustre viscose yarn, for example, was a method of retaining sulphur particles in the fibres by discontinuing the normal desulphurizing step during its manufacture. Although this yarn showed decreased lustre, due to scattering of light by the sulphur particles, it was impermanent and exhibited an unattractive "bloom". This method has been improved by dispersing, instead of sulphur, fine inorganic or organic particles and globules in cellulosic spinning solutions, for example, pigments, hydrocarbons, oils, etc. When inorganic compounds, such as titanium dioxide, silica, etc., are dispersed in cellulosic spinning solutions, they tend to cut the tread guides through which the yarns are led during the extrusion process, and in addition they weaken cellulosic yarns considerably. Hydro-55 carbons, emulsified with spinning solutions to de-

luster cellulosic products obtained therefrom, have the great disadvantage of being inflammable, while vegetable oils become rancid and form skin-irritating acids.

I have, unexpectedly, found that aliphatic silicon compounds possess properties which render them especially suitable as delustering agents for rayon products since they are very little inflammable and do not form irritating compounds. The following table depicts a number of aliphatic silicon compounds which may be used to deluster cellulosic products, although I wish to emphasize that my invention is not limited to these compounds since others may be used with equal success.

## TABLE

I. Derivatives having the structure  $R.SiH_3$ 

| Compound                             | Boiling or melting point | 20      |
|--------------------------------------|--------------------------|---------|
| Methyl-monosilane.....               | Degrees centi-grade      |         |
|                                      | 20-31                    |         |
| Ethyl-monosilane.....                |                          | 107     |
| Propyl-monosilane.....               |                          | 170-171 |
| Isobutyl-monosilane.....             |                          | 204-206 |
| Isoamyl-monosilane.....              |                          | 275-279 |
| Also higher molecular alkyl-silanes. |                          |         |

II. Derivatives having the structure  $R.SiH_2.OH$ 

| Compound                             | Boiling or melting point | 30      |
|--------------------------------------|--------------------------|---------|
| Ethyl-monosilanol.....               | Degrees centi-grade      |         |
|                                      | 154                      |         |
| Propyl-monosilanol.....              |                          | 203-208 |
| Isobutyl-monosilanol.....            |                          | 269-270 |
| Isoamyl-monosilanol.....             |                          |         |
| Also higher molecular alkyl-silanol. |                          |         |

III. Derivatives having the structure  $R.SiO.OH$ 

| Compound                                            | Form   | 40 |
|-----------------------------------------------------|--------|----|
| Silicon-acetic acid.....                            | Solid. |    |
| Silicon-propionic acid.....                         | Do.    |    |
| Silicon-butyric acid.....                           | Do.    |    |
| Silicon-caproic acid.....                           | Do.    | 45 |
| Also higher molecular silicon-fatty acid compounds. |        |    |

In addition, I have found that other aliphatic silicon compounds may be used for the purposes, set forth above, such as tetraethyl-monosilane, 50 triethyl-chloorethyl-monosilane, triethyl-acetoxy-ethyl-monosilane, halogenated monosilanes, tetrapropyl-monosilane, tripropyl-monosilane, tri-isobutyl-monosilane, triisoamyl-monosilane, tetraisoamyl-monosilane, triethyl-ethoxy-monosil- 55

ane, triethyl-monosilanol, siliconheptyl carbonic acid, triethyl-silicon chloride, triethyl-silicon bromide, silicon heptyloxide, tripropyl-monosilanol acetate, tripropyl-monosilyl bromide, bis-5 (tripropyl-monosilyl ether), triisobutyl-monosilyl bromide, trisoamyl-monosilyl bromide, bis-(triethyl-monosilyl ether), monosilyl derivatives of an oxy-compound, derivatives of monosilanol diols having the structure  $R.SiH(OH)_2$ , 10 methyl-orthosilicic acid-triethyl ester, ethyl-orthosilicic acid-trimethyl ester, ethyl-orthosilicic acid-triethyl ester, orthosilico-butyric acid-triethyl ester, orthosilico-isocaproic acid-triethyl ester, etc.

15

*Example*

About 1 to 30% of an aliphatic silicon compound is dispersed in, and/or emulsified with a cellulosic spinning solution, such as viscose and 20 cuprammonium cellulose, the aforementioned percentage being based upon the cellulose content of the solution. After uniformly distributing the delustering agent in the spinning solution, it is extruded through suitable spinning nozzles 25 into a conventional spinning bath. The solution may also be used for forming films or molding articles. Organic solvents, inorganic or organic pigments, etc., may be added to the spinning solutions besides silicon compounds. The 30 amounts of aliphatic silicon compounds, added to the solution, may be varied at will. In this manner more or less delustered rayon products may be obtained.

Modifications of my process will readily be 35 recognized by those skilled in the art, and I desire to include all those modifications falling within the scope of the appended claims. In these claims, the term "aliphatic silicon compound" is limited to such compounds which are 40 substantially water-insoluble and resistant to attack by alkalis and acids of such concentrations conventionally used in the rayon art.

I claim:

1. A spinning solution for the manufacture of 45 soft-lustre products comprising a solution of the group consisting of viscose and cuprammonium cellulose and a silicon compound having the structure  $R.SiH_3$ , in which R represents an alkyl radical, said compound being liquid and stable in said spinning solution.

2. As a new article of manufacture, regenerated cellulose containing a liquid finely dispersed silicon compound having the structure  $R.SiH_3$ , in which R represents an alkyl radical.

3. A spinning solution for the manufacture of 5 soft-lustre products comprising a solution of the group consisting of viscose and cuprammonium cellulose together with a substance of the group consisting of aliphatic silicon compounds having the structure  $R.SiH_3$ , in which R represents an 10 alkyl radical, aliphatic silicon compounds having the structure  $R.SiH(OH)_2$ , in which R represents an alkyl radical and aliphatic silicon compounds having the structure  $R.SiH_2.OH$  in which R represents an alkyl radical, said substance being 15 stable in said solution.

4. A spinning solution for the manufacture of 20 soft-lustre products comprising a solution of the group consisting of viscose and cuprammonium cellulose together with a silicon compound having the structure  $R.Si(OH)_2$ , in which R represents an alkyl radical, said compound being stable in said solution.

5. A spinning solution for the manufacture of 25 soft-lustre products comprising a solution of the group consisting of viscose and cuprammonium cellulose together with a silicon compound having the structure  $R.SiH_2.OH$  in which R represents an alkyl radical, said compound being stable in said solution.

6. As a new article of manufacture, regenerated cellulose containing a finely dispersed substance 30 of the group consisting of aliphatic silicon compounds having the structure  $R.SiH_3$ , in which R represents an alkyl radical, aliphatic silicon compounds having the structure  $R.SiH(OH)_2$ , in which R represents an alkyl radical and aliphatic silicon compounds having the structure  $R.SiH_2.OH$  in which R represents an alkyl radical.

7. As a new article of manufacture, regenerated cellulose containing a finely dispersed silicon compound having the structure  $R.SiH(OH)_2$ , in which R represents an alkyl radical.

8. As a new article of manufacture, regenerated cellulose containing a silicon compound 40 having the structure  $R.SiH_2.OH$  in which R represents an alkyl radical, said compound being finely dispersed throughout said cellulose.

RUDOLPH S. BLEY. 50